

# UNITED STATES PATENT OFFICE.

SAMUEL MANSFIELD JONES, OF NORTH ADAMS, MASSACHUSETTS, ASSIGNOR TO ARNOLD PRINT WORKS, OF NORTH ADAMS, MASSACHUSETTS, A CORPORATION OF MASSACHUSETTS.

## MERCERIZATION.

1,346,803.

Specification of Letters Patent.

Patented July 13, 1920.

No Drawing.

Application filed May 12, 1920. Serial No. 380,890.

To all whom it may concern:

Be it known that I, SAMUEL MANSFIELD JONES, a citizen of the United States, and a resident of North Adams, in the county of 5 Berkshire and State of Massachusetts, have invented new and useful Improvements in Mercerization, of which the following is a description.

This invention particularly relates to a 10 method of mercerizing cellulosic fibers of natural growth such as cotton or linen, when interwoven or intermingled with filaments of artificial silk known as viscose, while at the same time protecting such viscose filaments 15 from deleterious attack by the caustic alkali employed for mercerization.

Letters Patent No. 1,316,958, were granted to me September 23, 1919, for an invention which accomplished by its own particular 20 method therein set forth the novel utility just specified; but I have discovered that other methods are available for accomplishing the like ultimate result, and that among these is the method herein described which 25 involves the modification of the caustic alkali solution used for mercerization by introducing into it mono-acetyl-glycerin, which is otherwise known in chemical nomenclature as an acetic acid ester of glycerol or more 30 specifically monacetin.

For the purpose of the present invention I find it practically satisfactory to compose the mercerizing liquid by adding monacetin in the proportion of 181 grams to 819 grams 35 of an aqueous solution of sodium hydrate at 70° Twaddell. This proportion is not rigid; but if the ratio of the quantity of monacetin to that of the caustic alkali in solution at the hydrometric density stated is 40 much less than the ratio just indicated the viscose silk will not be adequately protected; and if such ratio is much greater the mercerizing efficiency of the caustic alkali thus modified will become impaired.

45 Glycerin which by reason of its chemical classification as a trihydric alcohol has also been named glycerol, may under reaction with glacial acetic acid at different temperatures be converted into three distinct esters 50 according as only one or each of two or all three of its hydroxyl groups become displaced by substitution therefor respectively of a corresponding number of acetyl groups, whereby either monacetin or diacetin or tri-

acetin results. But in conducting this process the obtainment thereby of monacetin alone without accompanying production of some diacetin or even of some triacetin requires careful precaution. Hence the commercial product known in the market as 55 acetin, and intended to be substantially monacetin, is likely to contain more or less diacetin and possibly triacetin, neither of which is capable of performing the functions of monacetin herein described. Nevertheless, the presence of such relatively small quantities of diacetin or of triacetin as may 60 ordinarily occur in commercial acetin does not seriously interfere with the efficiency of its largely preponderant monacetin in serving to modify the solution of caustic alkali for the protection of viscose silk associated in a composite fabric with natural cellulosic fibers which are subjected to the process of 65 mercerization.

70 Otherwise than such required modification of the mercerizing solution the treatment of the fabric into which mercerizable cellulosic fibers such as cotton or linen have been interwoven with viscose-silk filaments is substantially the same as that customarily employed in the mercerization of woven fabrics composed entirely of cotton including the usual means and mode of applying tension thereto for the prevention of shrinkage. 75

75 The employment of a mercerizing solution of caustic alkali which has been modified by the addition thereto of monacetin as hereinabove provided, enables the process of mercerization to be successfully practised 80 upon cellulosic fibers of natural growth such as cotton or linen, while at the same time the viscose silk filaments interwoven with these are effectively protected against injury from the caustic alkali; so that the 85 resulting product is expeditiously obtained without incurring the extra expense and labor required for separately mercerizing the cellulosic fibers in the yarn before interweaving the same with the viscose silk.

100 Manifestly also this invention although especially well adapted for the production of woven mixed goods of the kind hereinabove referred to, may likewise be practised upon yarns or other unwoven textile fabrics 105 which are composed partly of mercerizable cellulosic fibers such as cotton or linen and partly of viscose-silk filaments and which

are subjected to any well-known and acceptable process of mercerization suitable for imparting luster to the cellulosic components of a fabric thus constituted; except 5 only that instead of employing therein the old mercerizing chemical agent alone there is to be substituted therefor a solution of caustic alkali modified by the addition of monacetin, whereby injury to the viscose 10 components of the fabric is avoided.

I claim:

1. The method of treating textile fabrics composed of mercerizable cellulosic fibers intermixed with artificial silk filaments of viscose, for the purpose of mercerizing such cellulosic fibers without injury to the viscose silk, by subjecting the composite fabric thus constituted to a process of mercerization wherein the solution of caustic alkali 15 is modified by the addition thereto of monacetin.
2. The method of treating textile fabrics composed of yarn spun from mercerizable cellulosic fibers and interwoven with artificial silk filaments of viscose for the purpose of mercerizing the fibers of such yarn 20
- 25

without injury to the viscose silk, by subjecting the woven fabric thus constituted to a process of mercerization wherein the solution of caustic alkali is modified by the 30 addition thereto of monacetin.

3. The method of treating textile fabrics composed of cotton fibers intermixed with artificial silk filaments of viscose, for the purpose of mercerizing such cotton fibers 35 without injury to the viscose silk, by subjecting the composite fabric thus constituted, to a process of mercerization wherein the solution of caustic alkali is modified by the addition thereto of monacetin.

4. The method of treating textile fabrics composed of cotton yarn interwoven with artificial silk filaments of viscose for the purpose of mercerizing the fibers of such cotton yarn without injury to the viscose 40 silk, by subjecting the woven fabric thus constituted to a process of mercerization wherein the solution of caustic alkali is modified by the addition thereto of monacetin.

SAMUEL MANSFIELD JONES.